

## UNITED STATES PATENT OFFICE

2,223,524

## METHOD OF REFINING MINERAL OIL

Boris Malishev, Elizabeth, N. J., assignor of thirty and one-third per cent to Universal Development Corporation, New York, N. Y., and three per cent to John P. Nikonow, New York, N. Y.

No Drawing. Application August 12, 1939,  
Serial No. 289,919

3 Claims. (Cl. 196—39)

My invention relates to catalytic refining of hydrocarbons and has particular reference to refining of cracked gasoline.

This is a continuation-in-part of my patent application Serial No. 252,546, filed January 24, 1939, the latter being also a continuation-in-part of my application Serial No. 194,769, filed March 9, 1938, which matured into Patent No. 2,148,634; and Serial No. 205,724, filed May 3, 1938, which 10 matured into Patent No. 2,148,378.

As I disclosed in the foregoing and patents, my catalyst which represents a mixture of a mineral phosphate, superphosphate or Thomas slag with sulfuric acid or its equivalent calcined at a 15 temperature sufficient largely to expel free sulfuric acid but below red heat, can be also used for refining mineral hydrocarbon mixtures or their synthetic equivalents such as are obtained from coal carbonization, retorting bituminous 20 shales, Berguis, Fisher-Tropsh processes and others.

Although my process can be used for refining any types of hydrocarbon mixtures, including the less volatile petroleum fractions, such as kerosene and lubricating oils, its most important application is for refining cracked gasoline.

High octane gasoline obtained by high temperature vapor phase cracking is very difficult to refine. Sulfuric acid, the most commonly used 20 refining agent, is not suitable for refining this type of distillate; it gives treating losses of gasoline sometime as high as fifteen per cent (15%) and a considerable reduction of octane number. Several new refining agents were proposed, but 35 they were either too expensive, or involved certain difficulties such as rapid exhaustion, corrosion of equipment, poisonous effect, etc., which make practical application of the methods employing such agents impractical and sometime 40 even prohibitive.

My catalyst does not possess all these disadvantages and is cheaper than similar refining agents, such as phosphorus pentoxide or solid phosphoric acid catalyst.

45 My process in practice is carried out by passing hot oils or petroleum vapors through a heated bed of my catalyst. The refining action of my catalyst on cracked gasoline in most cases starts at 150° C., but is very slow and incomplete at that temperature. The optimum refining 50 temperature lies in the range of 250°—300° C. The optimum temperatures must be determined by every type of the crude oil. It is not advisable to proceed above 300° C., because at this temperature the cracking starts and produces col-

ored distillates; the gum formation also increases with the temperature. The time of contact with the catalyst depends on the difficulty encountered in effecting refining to the desired degree and varies from a fraction of a second to one or two minutes. To prevent material vaporization and drying out of the catalyst, sufficient superheated steam must be introduced into the catalytic chamber together with the crude gasoline. The amount of steam determined as water must be 5 about twenty per cent (20%) of the liquid gasoline.

Gum deposits rather rapidly if the distillate is totally in the vapor state. Hot liquid mineral oils dissolve the gum and prevent its deposition on 15 the catalyst. For that reason, in order to secure a good gum, free contact with the catalyst and prolong its life, I prefer to use medium pressures, such that a mixture of gas and liquid is formed. The pressure of about 200 pounds per square inch 20 is sufficient for this purpose. The treating losses with my catalyst are very small and are of an order of about 1.0% on cracked distillate. These losses are due exclusively to polymerization to 25 high boiling fractions.

*Example.*—A cracked unrefined gasoline of yellow color, poor induction period (two hours) and high copper disc gum content (600 mg. per 100 cc.) was pumped through a bed of my catalyst at 225° C. and at 200 pounds pressure with 30 twenty per cent (20%) steam. The product was redistilled to the desired end point.

The gasoline thus refined had a Saybolt color of 30+, copper disc gum of 10 mg. per 100 cc., and an induction period of ten hours. The anti-knock rating rose from 67 to 70 octanes. The 35 treating losses were about 1.0%. The life of the catalyst was 200 gallons gasoline per one pound of catalyst.

I claim as my invention:

1. A method of refining cracked gasoline, consisting in treating gasoline with a catalyst consisting of a solid calcined product of a mixture of a substance taken from the group consisting of a mineral phosphate, superphosphate and Thomas slag, with sulfuric acid, the treatment being conducted at a temperature from about 150 to 300° C. and at a pressure sufficient to maintain the liquid state.

2. A method of refining cracked gasoline, consisting in treating gasoline with a catalyst consisting of a solid product of a mixture of a substance taken from the group consisting of a mineral phosphate, superphosphate and Thomas slag, with sulfuric acid, calcined at a temperature suffi- 50 55

ciently high to largely expel free sulfuric acid but below red heat, the treatment being conducted at a temperature from about 150 to 300° C. and at a pressure of about 200 pounds per square inch.

3. A method of refining cracked gasoline, consisting in treating gasoline with a catalyst consisting of a solid product of a mixture of a sub-

stance taken from the group consisting of a mineral phosphate, superphosphate and Thomas slag, with sulfuric acid, calcined into a solid product, the treatment being conducted at an increased temperature but below cracking temperature and at a pressure sufficient to maintain the liquid state.

BORIS MALISHEV.